

# UNITED STATES PATENT OFFICE.

JEROME I. WOOD, OF WILMINGTON, DELAWARE, ASSIGNOR OF ONE-HALF TO  
WILLIAM M. WEST, OF SAME PLACE.

## METHOD OF MAKING FABRICS.

SPECIFICATION forming part of Letters Patent No. 431,426, dated July 1, 1890.

Application filed January 25, 1889. Serial No. 297,571. (No specimens.)

*To all whom it may concern:*

Be it known that I, JEROME I. WOOD, a resident of Wilmington, in the county of New Castle and State of Delaware, have invented 5 a new and Improved Method of Making Fabrics, of which the following is a specification.

The improved fabric, in the making of which the invention consists, is a parchment-like fabric, which can advantageously be used for 10 the purposes of ordinary parchment, for window-shades, or for other purposes where a strong, tough, pliable fabric is required.

The fabric is made in the following manner: For the body of the fabric any fibrous material may be employed, such as cotton, paper, wood-pulp, and the like. The fibrous material is first soaked in a bath or sizing composed of rosin soap dissolved in water. The rosin soap employed is the ordinary commercial rosin soap, which is composed of rosin, oil, or tallow, and soda or potash. The bath or sizing should be of about the consistency of milk when the fibrous material is introduced therein. When the material is thoroughly saturated with the sizing, it is hung in a warm room until it is nearly dry; but while still damp it is placed in a bath of chloride of zinc. In preparing the bath of chloride of zinc it is boiled down to a consistency of between 65° to 70° Baumé, and is used at a temperature of about 100° Fahrenheit. The material when subjected to this bath is dissolved to a certain extent, and the rosin soap permeates its pores and is thoroughly incorporated therewith. The resulting product is then passed directly over or between hot rollers. After this the material is allowed to cool, and is then washed in clear water to remove any surplus of the sizing and

chemicals. It is then hung in a hot room to 40 dry, and when dry it is given a coating of oil and is then passed through calenders. Any soft or limpid oil may be used, paraffine-oil being preferred. The fabric is then in condition for use. 45

The chloride of zinc turns the soap into an insoluble mass, closing all the pores of the material, thus making it capable of resisting dampness to a marked extent. Since no paint is applied to the fabric it is not liable to crack 50 or fade and it can be washed and ironed. The material will not show stains or grease-marks. On account of these qualities the fabric is especially fitted for use as window-shades, and it can be made at less cost than other good materials used for the same purpose. Its use, however, is by no means limited to this purpose. 55

The fabric can be made of any desired thickness, either by using a body fabric of the required thickness or by making it of two or 60 more plies.

I claim as my invention—

The herein-described method of preparing a fabric, which consists in, first, soaking a fibrous material in a bath of rosin soap; second, 65 drying the material; third, subjecting the material while yet damp to a bath of chloride of zinc; fourth, passing it over hot rollers; fifth, washing it; sixth, drying it; seventh, coating it with oil, and, lastly, passing it between calenders, substantially as set forth. 70

In witness whereof I have hereunto signed my name in the presence of two subscribing witnesses.

JEROME I. WOOD.

Witnesses:

HENRY C. CONRAD,  
THOMAS GIFFIN.